

## UNITED STATES PATENT OFFICE

HENRY L. CROWLEY, OF EAST ORANGE, AND ROBERT M. CROWLEY, OF JERSEY CITY, NEW JERSEY, ASSIGNORS TO HENRY L. CROWLEY & CO. INC., OF EAST ORANGE, NEW JERSEY, A CORPORATION OF NEW JERSEY

## CERAMICS

No Drawing.

Application filed March 2, 1929. Serial No. 344,091.

This invention relates to ceramics and more particularly to a method of eliminating corrosive effects in ceramic materials.

An object of the invention is the provision of a method which will secure the elimination of such corrosive effects.

A further object of the invention is to provide a method in the production of ceramic material which will provide a product free from chemical reaction.

A further object of the invention is to provide a method of purifying the material utilized in the fabrication of ceramic products.

Further objects of the invention will appear more fully hereinafter.

The invention consists substantially in the method of procedure and the product obtained thereby, all as will be more fully hereinafter set forth and finally claimed in the appended claims.

In ceramic materials where a metal in a completely fabricated structure is employed in contact with the ceramic material, such for example as a porcelain-like tube with one or more orifices through which a metal extends, it has been found that when the completed structure is subjected to heat a chemical reaction between the tube and the metal occurs resulting in the corrosion of the metal

30 having various deleterious effects on the completed structure or the operation thereof. For example, in the radio vacuum tube industry, and particularly in the so-called alternating current tubes where a heater element is employed as the cathode of the radio tube, it is customary to employ a ceramic tubing as the heater element, which tubing is provided with one or more (usually two) hair-like orifices extending therethrough and

40 through which the hairpin or other shaped incandescent filament passes. Corrosion thus occurring in the hair-like incandescent filament (usually but not always formed of tungsten or other rare earth metal) has the bad effect of imparting a short life for the filament in use and hence a short life for the radio vacuum tube of which it forms a part. We have discovered that this cause for short life of the filament, viz: corrosion thereof

50 caused by chemical reaction between the ce-

ramic tubing and the filament can be eliminated by the special treatment which forms one phase of the substance of our present invention.

We have discovered that the principal if not the entire cause of corrosive effects of metals in contact with ceramic materials has been due to the presence of alkali in the respective materials. In accordance with our invention, therefore, we eliminate the alkali from the materials forming the ceramic product, as well as from the metal structure or the associated elements forming part of the completed article of manufacture.

For the purpose of disclosing our invention to enable those skilled in the art to utilize the same and readily appreciate the commercial, scientific, and practical advantages thereof, we will adhere to the illustration hereinabove given, to wit: a radio vacuum tube, but we wish it to be understood that our invention in its broad scope is not to be limited or confined to any particular application or utilization as the advantages thereof, now made apparent, can be readily appreciated and utilized in any art where deleterious or undesirable corrosive effects between a ceramic product and an associated metal are sought to be obviated.

In constructing a heater element of a radio vacuum tube operating on alternating current in accordance with our invention we choose materials which are as free as possible from alkali. By this we do not mean that it is necessary to obtain one hundred percent purity, though it is desirable. Small traces of alkali may be present without an undesirable deleterious effect but ordinary precautions in the selection of material, as well as in the treatment forming part of our invention, will permit the substantial attainment of our present invention.

In producing the ceramic tubing we take the selected powdered material and add thereto a non-alkali binder, such as beryllium oxide or any such similar material which may be selected in accordance with the diagonal law of the periodic table which forms the subject matter of the copending application Serial No. 332,555 filed January 14, 1929.

Binders other than beryllium oxide may be employed, notably those that burn out in the final firing. However, beryllium oxide may be employed as a binder and, if employed, does not burn out in the final firing but fluxes, thereby adding strength and rigidity to the ultimate product. The powdered ceramic material and the binder are each subjected to a heat, preferably by baking them in a furnace, at a temperature below their fusion point and for a period which is dependent upon the particular material being baked and the degree of purity desired. This effects a burning out of all the impurities sublimable at the temperature at which the materials are being subjected, and causes a coagulation of all other impurities, which may be readily sifted out of the powdered materials being treated. The binder and the ceramic material, both in the powdered form, are then mixed and extruded under pressure into the desired form determined by the die of the extrusion press. The material is then subjected to machining, where desired and necessary.

These various steps are described in more detail in the copending application above identified, the foregoing description being deemed to be sufficient for the purposes of the present case.

The product thus obtained is finally fired, i. e. subjected to heat, for example baked in a furnace, in a strongly reducing atmosphere, i. e. more gas (CO) than air. In other words, it is desirable to eliminate the presence of all free oxygen. By this means the occluded gas in the materials being subjected to the heat treatment will consist largely, if not entirely, of the gas in which the alkali was reduced, viz: carbon monoxide (CO), to the exclusion of free oxygen. By reason of this heat treatment, for example in the case of the radio vacuum tube, when the tube is in use excess heating releases from the heater element carbon monoxide and no oxygen and therefore the metal of the filament (for example tungsten where that metal is used) is not oxidized. In fact, due to the affinity of carbon monoxide and any free oxygen which may be present in the tube irrespective of its source, the carbon monoxide will combine with such free oxygen and form carbon dioxide, an inert gas, with the result that the heater element produced in accordance with our invention in itself acts in use as a "getter."

In the vacuum tube art it will be readily seen with these elements the use of the alkali getters, such as potassium, etc., at present employed with their incident deleterious effects on the metallic filament while at the same time enabling the obtaining of the "getter" action of such vaporizable metals, for which purpose, without knowledge of the deleterious effects of alkali, such materials

were originally proposed and have been used in this and allied arts. However, we have found that in forming the ceramic material if a small percentage of magnesium oxide in powdered form is used (ten per cent or less) on final firing part of the occluded gas in the ceramic tube comprises magnesium oxide with the result that both a "getter" and a "keeper" action are obtained in the tube.

Many modifications and changes in details will readily occur to those skilled in the art without departing from the spirit and scope of our invention as defined in the claims, but having now set forth the objects and nature of our invention and having described a method and a product obtained in accordance therewith, both embodying our invention, what we claim as new and useful and desire to secure by United States Letters Patent is:

1. The method of producing a non-corrosive ceramic which comprises extruding under pressure a pulverized material and binder free from alkali and baking the same, said material and binder being freed from alkali by heating below the fusion temperature.

2. The method of producing a non-corrosive ceramic which comprises extruding under pressure a pulverized material and powdered beryllium oxide and baking the same.

3. The method of producing a non-corrosive ceramic which comprises extruding under pressure a pulverized material and binder previously freed from material having an alkali reaction at high temperatures and baking the same at a temperature sufficiently high to burn out the binder.

4. The method of producing a non-corrosive ceramic which comprises extruding under pressure a pulverized material and powdered beryllium oxide and baking the same at a temperature sufficiently high to flux the beryllium oxide.

5. The method of producing a non-corrosive ceramic which comprises subjecting a powdered material to heat below its fusion temperature to purify the same and extruding the purified material under pressure and baking the same.

6. The method of producing a non-corrosive ceramic which comprises subjecting a powdered material and a binder to heat below their fusion temperatures to purify them, mixing the material and binder, extruding the mixture under pressure, and finally subjecting the extruded product to heat to flux the binder without fusing the powdered material.

7. The method of producing a non-corrosive ceramic which comprises subjecting a powdered material and a binder to heat below their fusion temperatures to purify them, mixing the material and binder, extruding the mixture under pressure, and finally subjecting the extruded product to heat at a

temperature sufficiently high to burn out the binder without fusing the powdered material.

8. The method of producing a non-corrosive ceramic which comprises subjecting a powdered material free from alkali to heat below their fusion temperatures to purify the same, mixing the material with an alkali free binder similarly purified, extruding the material under pressure, and finally baking the extruded product.

10. 9. The method of producing a non-corrosive ceramic which comprises subjecting a powdered material free from alkali to heat below their fusion temperatures to purify the same, mixing the material with an alkali free binder similarly purified, extruding the material under pressure, and finally baking the extruded product at a temperature sufficiently high to burn out the binder.

20. 10. The step in the process of producing a ceramic product which comprises purifying the ceramic in powdered form by heating it below its fusion temperature, and firing the product in a strongly reducing atmosphere of gas to cause any free oxygen to be replaced by the reducing gas.

30. 11. The step in the process of producing a ceramic product which comprises initially purifying the ceramic in powdered form by heating it below its fusion temperature, firing the product in a gaseous reducing atmosphere free from free oxygen to cause the free oxygen in the ceramic to be replaced by the reducing gas.

35. 12. The step in the process of producing an alkali-freed ceramic product which includes the step of firing the product in a gaseous reducing atmosphere free from free oxygen to cause any free oxygen in the ceramic to be replaced by the reducing gas.

40. 13. The step in the process of producing a ceramic product which comprises firing the product in an atmosphere of carbon monoxide to cause any free oxygen in the ceramic to be replaced by carbon monoxide.

45. 14. The step in the process of producing an alkali-freed ceramic product which comprises firing the product in an atmosphere of carbon monoxide to cause any free oxygen in the ceramic to be replaced by carbon monoxide.

50. 15. A ceramic formed of a compressed and baked powder with its occluded gases consisting substantially entirely of carbon monoxide.

55. 16. A ceramic formed of a compressed and baked powder containing in part a powdered form of a metal having "getter" properties.

60. 17. In the art of manufacturing a metal filament and a ceramic adjunct thereto capable of being used at high temperatures without corrosion of the filament, the method which comprises powdering a metal oxide, heating the powdered oxide to a temperature below its fusion point to separate out mate-

rials having an alkali reaction at high temperatures, sifting out the alkali freed powder and mixing it with a non-alkali binder, extruding the mixture under pressure to tubular form, and threading said filament through said tubular member.

70. 18. The method according to claim 17 in which the extruded tubular member is baked before threading of the filament to flux the binder.

75. 19. The method according to claim 17 in which the powdered oxide is mixed with a non-alkaline binder of beryllium oxide.

80. 20. The method according to claim 17 in which the extruded tubular member is baked before threading of the filament to flux the binder below the fluxing temperature of the powdered metal oxide.

85. 21. The method according to claim 17 in which the extruded tubular member is baked before threading of the filament in a reducing gaseous atmosphere to cause the said gas to replace the free occluded gas in said member.

90. 22. The method of manufacturing a heater element for radio tubes which comprises selecting a powdered metal containing substantially no impurities which have an alkali reaction at high temperatures, mixing with said powdered metal a small percentage of a metal having getter properties, extruding said mixture to tubular form, baking the extruded member and threading through said extruded member a metal filament.

95. 100. 23. The method of manufacturing a heater element for radio tubes which comprises selecting a powdered metal containing substantially no impurities which have an alkali reaction at high temperatures, mixing with said powdered metal a small percentage of a powdered oxide of a metal having getter properties, extruding said mixture to tubular form, baking the extruded member and threading through said extruded member a metal filament.

105. 110. 24. The method according to claim 23 in which the metal having getter properties consists of powdered magnesium oxide.

115. In testimony whereof we have hereunto set our hands this 21st day of February A. D., 1929.

HENRY L. CROWLEY.  
ROBERT M. CROWLEY.

12.

125

129